

## UNITED STATES PATENT OFFICE

PHILIP W. CODWISE, OF KENMORE, NEW YORK, ASSIGNOR, BY MESNE ASSIGNMENTS,  
TO CERTAIN-TEED PRODUCTS CORPORATION, A CORPORATION OF MARYLAND

## FELT

No Drawing.

Application filed August 19, 1926. Serial No. 130,361.

This invention relates to and has as an objective, among others, the efficient and inexpensive manufacture of improved and novel fibrous products.

This application is a continuation in part of my co-pending application Serial No. 21,727 filed April 8, 1925 and is also a continuation in part of my copending application Serial No. 42,316, filed July 8, 1925.

10 The nature of the invention may be best understood by reference to one exemplification thereof relating to vegetable and wood fibre having novel and advantageous characteristics and to one illustrative use of such fibre.

In the present exemplification of the invention, vegetable fibre, which is advantageously in the form of wood chips (pine chips for example) is partially disintegrated by 20 treatment which partially removes or loosens the lignins, resinous and pectic substances which occur with the bundles of fibre to make up the wood structure. This partial removal or loosening of these encrusting and binding substances preferably does not result in a reduction of the wood to ultimate cellulose fibre nor substantially so, but preserves the bundles of fibres with their characteristic length and strength, rendering them soft and capable of 30 interlacing and felting well.

Such partial disintegration of the wood structure may be advantageously effected in the present instance, by cooking the chips under pressure in a relatively weak alkaline solution. To assist in disintegration and to facilitate the action of the alkali on the wood structure, the wood chips may be given a preliminary treatment which promotes the penetration or impregnation of the wood by the 40 alkaline solution. For example, such preliminary treatment may consist in steaming the wood chips (using one hundred parts of pine chips as a convenient illustration) in a digester for about three-quarters of an hour.

45 The wood may be provided in convenient chip form by the usual chipping machine, the chips in such cases being about one inch in length.

The treatment with steam apparently promotes the rapid impregnation of wood with 50 an alkaline solution, which impregnation

should take place immediately after steaming. Thorough impregnation is obtained by soaking in a solution containing, for example, sodium hydroxide for a period sufficient to effect the desired result.

If desired the above mentioned preliminary steps can be omitted and the proper amount of alkali in suitable solution may be introduced directly into the digester preparatory to the cooking period which will now be 55 described.

The chips are then subjected to an alkaline cook, such as with sodium hydroxide in about 60 seven percent proportion. The amount of alkali is based upon the bone dry weight of 65 the chips—the amount being determined by what is necessary under proper treatment to secure adequate disintegration of the fibre encrusting substances and the desired condition of the fibre—but usually falls within the 70 limits of four to twelve percent. Sodium hydroxide is preferable as an alkali because of its efficiency, yet other chemicals, such as sodium sulphite, sodium carbonate, calcium hydroxide may be used. However, a low 75 percentage of alkali is important in that it assists in the peculiar disintegration of the wood, and further reduces the chemical cost so that a chemical recovery system may be unnecessary. While any wood which will 80 respond to treatment to secure the desired fibre properties may be used coniferous woods such as pine, fir, hemlock, cedar and spruce, are 85 advantageous because of low cost and character of fibre produced.

The chips are cooked in a digester under steam pressure of about 100 pounds per square inch pressure and at a temperature of about 160° C. Where the chips are not subjected to the preliminary softening and impregnation treatments, the time consumed in cooking is somewhat longer—from six to twelve hours—and the alkaline concentration in the digester (per 100 parts of wood) should be from 4 to 10 parts by weight of sodium hydroxide in about 300 parts by weight of water. If the chips are given a preliminary steaming the time consumed in cooking is lessened by several hours.

After the cooking has been carried to the

proper point, the chips are removed from the digester and washed. They are now in such a state that they may be reduced to the proper fibre condition by mechanical shredding, washing, and beating with water. The shredding is conducted so that the bundles are separated from each other, without the bundles themselves being shredded to any material extent. While other suitable means 5 may be employed, I have found a swing hammer pulverizer most efficient, whereby the fibres are beaten in air, with the swing hammers setting up an air circulation to remove the beaten bundles. The degree of shredding 10 is regulated by the exit door of the machine. The resulting product has peculiar and distinctive characteristics, and is suited for many uses in which wood fibre has not heretofore been adapted or satisfactory. The 15 20 partial disintegration of the wood structure converts the long sliver-like formations of the wood into irregular composite fibre bundles in which the fibres are held together only sufficiently to give the bundle the desired 25 30 length and strength but not firmly enough to impair its flexibility and softness nor to interfere with its intertwining and felting characteristics. Contributing to the latter characteristics are the numerous loose and free 35 40 ends of the individual fibres or groups of fibres which project from the body of the fibre bundles. Wood fibre product is a fibrous mass containing long slender fibrous aggregates, each of which contain a various 45 50 number of fibres. These aggregates vary from the length of an individual fibre to bundles of these fibres some of which are about one and one-half inches in length. The average length of a bundle is approximately 55 60 one-half inch with the average width varying from that of an individual fibre to one sixty-fourth of an inch. There will be a certain proportion of short fibres which intermingle with and bind the bundles together. 65 After the beating treatment, the stock may be put to any desired use. By way of illustration, it may be run directly into an ordinary felt machine, such as the Fourdrinier or cylinder type, and manufactured into a 70 75 strong, soft and porous felt. Contributing to the porosity of the sheet is the characteristic coarseness of the fibre bundles which will strongly intertwine and felt without being compressed into a dense sheet. 80 85 Among other characteristics, the felt is remarkably permeable and absorbent, and may be advantageously used as a vehicle for various liquids and saturants to provide whatever prepared product is desired. For example, 90 95 as an element in prepared roofing, the felt will absorb from 200% to 250% of its weight of saturating asphalt or the like (as against about 180% in the case of ordinary rag felt), and it is easily possible to make the percent- 100 105 age of absorption even higher.

The distinctive properties of the felt are manifest not only in its absorptive capacity but in rapidity of absorption. Contributing thereto are the characteristic porosity of the felt and the capillarity of the bundles of 70 75 fibres largely making up the felt,—the capillarity probably being produced by the capillary spaces between, within and around the loosened fibres left by the removal or partial removal of the encrusting substances associated with the fibres in the normal wood structure. The absorptive capacity of the felt may be wholly controlled and varied by the degree of subdivision of the bundles, or it may be controlled and varied by mixing 80 85 with the stock varying quantities of adulterating stocks such as rag or waste paper stocks which are short fibred and will fill the voids between the bundles, thereby having the effect of reducing the absorptive capacity. Any proportion of waste stock may be used 90 95 with the wood fibres, depending on the degree of porosity desired for the felt. I have found medium weight felt composed of substantially 75% wood stock and 25% waste stock to be well adapted for ordinary purposes. It is to be understood, however, that the waste stock is not an essential ingredient, and, if used, can be used in any proportion desired. The absorptiveness may also be 100 105 regulated to some extent by the degree and duration of compression to which the felt web is subjected in the felt machine, although this novel wood fibre, unlike other fibre stock, has the ability to intertwine and felt naturally without material compression, thereby making it possible to make a very open and porous felt.

Obviously the invention is not limited to the details of the exemplification thereof herein described, since these may be variously modified. Moreover it is not indispensable that all features of the invention be used conjointly since various features may be advantageously employed in different combinations and subcombinations. 110

Having described one embodiment of my invention, I claim:

1. The process of producing a fibre product from wood which consists in modifying by incomplete chemical treatment the substances naturally encrusting and binding the fibres of the wood while not completely releasing in said treatment the fibres from each other, and subdividing the wood for the most part into bundles of long fibres maintaining approximately the natural arrangement of the fibres with respect to each other in the bundles. 115 120

2. The process of producing a fibre product which consists in the partial disintegration of wood by cooking under pressure in an alkaline solution to partially loosen but not completely remove the encrusting substances associated with the fibre in the wood structure whereby the fibres are imperfectly 125 130

- retained in their natural arrangement, and shredding said wood to produce for the most part flexible bundles of fibres in such arrangement of substantial strength and capable of firmly felting together. 5
3. The process of producing an absorbent fibre product from wood which is characterized by chemically modifying the encrusting substances associated with the wood 10
- 10 fibres to provide increased capillarity of said encrusting substances partially retained between the fibres, and then mechanically shredding the wood to produce masses consisting for the most part of bundles of fibres 15 bound by said modified substances in approximate natural arrangement.
4. The method of making fibre, which is characterized by cooking wood material with 4% to 14% of its weight of alkali to soften it, and shredding the same into a mass of bundles of fibres, in which mass the major portion of the bundles is in the form of flexible threads containing fibres in their natural relationship. 20
- 25 5. The process of producing wood fibre consisting in steaming wood material, cooking the same under pressure at an elevated temperature with an alkali to partially disintegrate the encrustations, and shredding the remaining structure into a mass of fibre bundles, in which mass the major portion of the bundles is in the form of flexible threads containing fibres in their natural relationship.
- 25 6. The method of making felt which comprises cooking under pressure wood chips with 4% to 14% of their weight of alkali to soften them and incompletely release the bond between individual fibres, shredding the chips for the most part into flexible fibre bundles and matting the same into sheets, the fibre bundles containing the fibres for the most part in their natural relationship. 30
7. The method of making dry felt which 45 comprises chemically softening the bond between fibres of wood insufficiently to release the fibres from each other in their natural arrangement, separating the wood into bundles of said incompletely released fibres, and matting said bundles into sheets, the fibre bundles containing the fibres for the most part in their natural relationship. 50
8. The method of making felt which 55 comprises cooking wood with weak sodium hydroxide solutions to weaken but not completely remove the bond between the fibres, shredding the resulting fibrous material for the most part into fibre bundles of irregular size having the fibres therein retained in 60 part at least in their natural relation, and matting the same into sheets.
9. The process of making felt of predetermined permeability which consists in forming a felt stock by shredding into bundles of wood fibres wood treated chemi- 65 cally incompletely to remove the bond between the fibres so as to leave the fibres in the bundles in approximate natural relation to each other, whereby when felting an open felt is produced, and controlling the permeability of the felt by mixing with the felt stock a quantity of short fibre which partially fills the voids between the bundles of the felt stock. 70
10. The process of making absorbent felt 75 which is characterized by partially disintegrating wood by treatment with limited amounts of alkaline chemicals to incompletely loosen the encrusting substances so as to release fibre ends while maintaining the fibres bound in approximately natural relation, reducing the treated wood to shreds consisting of irregular bundles of fibres so bound, mixing the shreds with water and forming a wet felted web from such shredded stock, and controlling the porosity of the felt web by the degree and duration of pressure on said web. 80
11. An intermediate wood product consisting of wood fibres and their natural bonding 85 encrustations for the most part in the form of bundles of fibres, the encrustations being in a chemically modified state while maintaining a bond between the fibres in the bundles at least partially to retain the natural arrangement of the fibre in the bundles. 90
12. As an article of manufacture, a partially cooked and disintegrated absorbent wood product comprising for the most part bundles of individual fibres substantially 95 longer and stronger than the individual fibres, said fibres being held together in the bundles by the natural encrusting substances associated therewith substantially in their relation as in the wood structure, said encrusting substances being in a chemically partially disintegrated state whereby the fibre bundles are absorbent by reason of the capillary spaces provided by the partially disintegrated encrusting substances. 100
13. As an article of manufacture, a shredded vegetable fibre suitable for felt comprising for the most part bundles of chemically treated wood fibre in which the individual fibres of the bundles substantially retain their natural positions in the bundles and are held together by a part of the encrusting substances naturally associated therewith in the wood structure to form the shreds, the balance of said encrusting substances being loosened or removed by the chemical treatment to loosen or release parts of the individual fibres, thereby giving the shreds flexibility and good felting qualities. 110
14. As an article of manufacture, a felt of predetermined permeability comprising in combination an open felt structure formed for the most part of long fibre bundles composed of wood fibres held together substantially in their natural arrangement by the natural encrusting substances chemically 115
- 120
- 125
- 130

modified to soften the bundles, the pores or voids between the bundles in such felt structure being partially filled with other material to control the effective size of the voids and the permeability of the felt structure.

15. As an article of manufacture, a flexible sheet of material possessing absorption properties composed of coniferous wood fibres disintegrated for the most part into masses of long fibre bundles, and waste paper stock, felted together, said fibre bundles having the fibre encrusting substances chemically softened but bonding the fibres in the bundles in substantially their natural arrangement.
16. As an article of manufacture, a sheet of absorbent felt composed of coniferous wood disintegrated for the most part into bundles of the wood fibres, and ordinary rag felt fibres felted with the bundles of wood fibres, said bundles of fibres having the natural bonding encrustation of the fibres chemically modified but retaining sufficient bond between the fibres to preserve substantially the arrangement of the fibres in the bundles.
17. As an article of manufacture, a flexible sheet of fibrous material composed of wood disintegrated for the most part into bundles of fibres in substantially their natural arrangement held together by their natural bond chemically modified to increase the absorptive capacity of the bundles, said fibres being felted together to form a porous sheet capable of absorbing at least twice its own weight of a waterproofing or filling saturating material.

In testimony whereof, I affix my signature.

PHILIP W. CODWISE.

40

45

50

55

60

65